

No. 885,328.

PATENTED APR. 21, 1908.

B. E. ELDRED.  
PROCESS OF OXIDIZING ORES.  
APPLICATION FILED FEB. 8, 1906.



WITNESSES:

Ross Barnes  
A. M. Houghton.

INVENTOR.

Byron E. Eldred  
BY  
Marble & McElroy.  
ATTORNEY.

# UNITED STATES PATENT OFFICE.

BYRON E. ELDRED, OF BRONXVILLE, NEW YORK, ASSIGNOR TO COMBUSTION UTILITIES COMPANY, OF NEW YORK, N. Y.

## PROCESS OF OXIDIZING ORES.

No. 885,328.

Specification of Letters Patent.

Patented April 21, 1908.

Application filed February 8, 1906. Serial No. 300,128.

*To all whom it may concern:*

Be it known that I, BYRON E. ELDRED, a citizen of the United States, residing in Bronxville, in the county of Westchester 5 and State of New York, have invented a certain new and useful Process of Oxidizing Ores, of which the following is a specification.

This invention relates to processes of treating ores and consists in a method of regulated roasting of galena and similar sulfid ores by means of draft currents of diluted air delivered through masses of such ore; all as more fully hereinafter set forth, matters of novelty being particularly pointed 15 out in the appended claims.

Galena and similar fusible sulfids are roasted with great difficulty by the processes now in use, particularly when rich ores and concentrates are treated. Oxidation of lead sulfid is a heat developing or exothermic 20 reaction and tends to be self-accelerating in a measure, becoming violent and uncontrollable when free access of ordinary air is permitted. But as galena is readily fusible, such a violent reaction melts it superficially, 25 rendering access of air to the interior of a lump impossible and producing uneven burning. Further, in such irregular roasting, there is a tendency for a portion of the sulfid 30 to oxidize to sulfate which then reacts with another portion of unchanged sulfid to produce sulfur dioxid and metallic lead according to a well known reaction. For these reasons, in the ordinary methods of roasting rich ore there must be a constant supervision 35 of the charge by highly skilled furnace men to prevent irregular roasting with the result of unchanged sulfids appearing in the roasted ore and to prevent the formation of metallic 40 lead in the furnace.

Regulation of the rate of burning to prevent these detrimental results is not possible by the ordinary means and methods used with other ores. Mechanical rabbling, as in 45 continuously operating reverberatories, is not very feasible since the readily fusible galena gums on rabbling tools. Hand rabbling while more practicable is heavy, exhausting work and requires high skill on 50 the part of the operator. Further, unless great care be exercised to prevent fusion, only the surface layers can be rabbled successfully. The process is very slow and the ore is apt to come out of the furnace, if 55 successfully roasted, in a fine pulverulent

state which is highly undesirable for most purposes and particularly where the calcines are to be used in the smelting furnace. Dusty materials of this character impede the blast in the furnace and are blown out of 60 the stack, causing great losses. For this reason smelting furnaces often briquet such dusty calcines with lime. This is expensive and not very satisfactory as the bricks frequently prove too weak to sustain the burden of the furnace.

In the prior art, efforts have been made to obviate the stated inconvenience by admixing greater or less quantities of inert materials, or diluents, such as lime, sand, etc., 70 with the rich ores or concentrates to restrain the violence of the reaction and insure the production of porous, thoroughly roasted calcines. In other words, the rich ores have been converted into poor, it being considered 75 less inconvenient to add an impurity which must afterwards be removed with some trouble and expense, rather than endeavor to contend with the fusibility and heat-evolving tendencies of such rich ores. I have, 80 however, discovered that the diluent or inert material may as well be added to the oxidizing medium or air, used in roasting, as to the ore itself. Obviously this is much more 85 convenient and much less expensive, both in the treatment itself and in subsequent treatments, while many other advantages are gained. The reaction is under perfect control which is not the case when the ore itself is diluted, since the composition of the draft currents can be instantly changed by the regulation of a valve or two.

Rapidity of combustion is a phenomenon depending as much upon the relative mass or concentration of the oxidant as upon that of the substance oxidized; and it may be varied by varying the composition of either. For many purposes, as in this art, it may be said that air is, so to speak, too concentrated; it gives rise to reactions too violent and uncontrollable in their nature. On the other hand, if it be diluted, the reacting mass of the oxygen is lessened and under the laws of mass action or the "phase rule," its reactivity lessens more than corresponds to the sheer dilution. This fact I have discovered may be very advantageously applied in the treatment of galena. It is merely necessary to dilute the draft current supplied to the mass of roasting ore with any inert gas in order to 110

slow down the violence of the oxidation to any desired degree. As cheap and convenient for this purpose, I regard the products of combustion; preferably from a fuel burning furnace, although the products from sulfid roasting furnaces may be used; *i. e.*, gaseous mixtures containing sulfur dioxid. Both may of course be used in special cases. Ordinarily however, when desiring to roast 10 galena and similar sulfids to oxid, I prefer to use the products from fuel burning furnaces. Such products ordinarily consist of a mixture of carbon dioxid and nitrogen, with a little steam at times and some unburned gases 15 or air. Products richer in carbon dioxid may be obtained from lime and cement kilns and other furnaces treating carbonates. Steam I do not regard as an inactive diluent in the sense of the permanent gases mentioned for 20 the reason that it has great reactive powers with sulfids, sulfites, etc., but in some embodiments of my invention a modicum may be used together with the diluents stated in the draft current. It is especially useful in 25 cases where an oxid as free as possible from sulfate is required since it tends to decompose intermediate sulfites which may be formed. On the other hand, where it is desired to burn galena to lead sulfate, as in the 30 production of a cheap white lead substitute, steam is to be avoided and the diluent gas is preferably derived from sulfur burning furnaces, sulfur dioxid having a specific action favoring the production of sulfates in this 35 method of roasting.

While the draft currents described may be passed over the sulfid to be roasted or brought into contact therewith in any of the well known ways, in the present specific embodiment of my invention I prefer to pass them through a body of the ore in the manner hereinafter described. For this purpose, apparatus of the type shown in the accompanying drawing can conveniently be used although 45 I do not in any way restrict myself to the use of any particular type of apparatus, my invention being susceptible of being carried out in many other forms of apparatus.

In the apparatus shown in the accompanying drawing, 1 designates the vessel in which the treatment is conducted, the same comprising, in the form shown, a vessel of the general nature of a shallow converter, mounted upon trunnions 2 so as to be capable of 55 being tilted as hereinafter described, and having a perforate false bottom 3, and a hood 4, the latter arranged to lift and having a telescopic or other suitable connection with a stack 5. The said converter is provided 60 with means for supplying to it, and for passing through the material in treatment therein, a draft current of any desired composition and temperature, such draft current being supplied by means of a blower 6 connected by a pipe 7 to one of the trunnions 2,

which is hollow, and is connected by a passage 8 to the chamber 9 beneath the perforate false bottom 3 of the converter. The inlet of this blower is connected to means for supplying hot and cold air, products of combustion, steam or aqueous vapor, the products of the combustion of sulfur, etc. For this purpose I have shown an ordinary furnace 10, which may be of any type and may be used for any purpose, even one foreign to the present process, the only function of this furnace, so far as this process is concerned, being to supply products of carbon combustion and to heat the entering air, both of which operations it may obviously perform 75 while likewise performing a main function not in any wise related to the process herein described; and for the same purpose of supplying ingredients of the draft current to the blower I have shown a pipe 11 leading from the offtake of said furnace to the blower and provided with a regulating valve 12; an air supply pipe 13 passing for a portion of its length through a heated region, as for example the offtake of furnace 10, and hence constituting an air heater; a pipe 14 connected to a suitable source of supply of products of sulfur combustion, not shown; a cold air inlet 15, and a source of supply of aqueous vapor (steam, or water in the form of a spray or 90 other form suitable to permit ready absorption by the draft current) 16; these several pipes being provided with suitable regulating valves 17, 18, 19 and 20, respectively. By proper regulation of these valves a draft 95 current of any desired constitution may be obtained.

Valves 17 and 19, controlling respectively the admission of hot and cold air, further constitute convenient means for regulating 105 the temperature of the draft currents. By provision of this plurality of sources of gases of different characters, I make it possible to regulate exactly conditions within the sulfid roasting chamber. With admission of a 110 draft current composed of cold air and products of combustion, the oxidation may be checked while with the same relative proportions of heated air and products of combustion in a draft current it may be accelerated. The admission of water to the draft current 115 of air and products of combustion, cools it still further in cases where a cold but oxidizing draft current is desired, while steam does not lower the temperature so much. The 120 steam or water vapor while in no sense a diluent gas, is nevertheless frequently very convenient as affording an additional means for completing the expulsion of oxidized sulfur as it has a specific dissociating action 125 upon sulfites and similar salts.

Steam is a very suitable form of aqueous vapor to use; but as to supply steam generally requires the presence of a steam boiler, which is not always convenient or desirable, 130

and since the entering draft currents take up water readily, I may introduce the water in the form of a spray or in any other suitable manner so that the water will be taken up by 5 the draft current as aqueous vapor.

In using my process for the roasting of lead sulfid in this form of apparatus, the converter may be preliminarily heated and the reaction started by placing a layer of char- 10 coal or other fuel on the false bottom and getting it well alight by means of an air draft current, the valves being suitably adjusted for this purpose. A layer of the galena is then 15 added and when the oxidation begins, the converter is filled to a suitable depth. As the oxidation progresses and heat develops it is restrained by closing valve 19 or 17 somewhat and opening valve 12, thereby diluting the air draft with stack gases from 20 the furnace. As the reaction proceeds, the proportion of diluent gas is increased until the exothermic tendency slackens when it is again decreased. The proportions are at all 25 times during the early part of the roasting so adjusted that while oxidation proceeds freely the temperature does not rise to a point where the galena would fuse or clinker. It is desirable for even roasting that the 30 galena be kept porous until nearly all the oxidation is complete, thereby permitting the permeation of oxygen throughout the interior of all lumps of ore. The draft however, may be forced to a degree hitherto 35 wholly unknown in this art for, since the oxidation nowhere becomes violent, the oxidation may be safely permitted to take place in all parts of the mass of ore undergoing treatment. In other words, instead of treating 40 a superficial shell of material as in ordinary furnaces where the mass is mixed from time to time by hand labor, the porous mass may be simultaneously treated throughout. So, although the generation of heat is 45 repressed and the possibility of clinkering obviated, yet forced working is practicable.

When desiring to make oxid with little or no sulfate as is usually desirable, the products of combustion from the reverberatory alone are used, but where sulfate is desired a 50 modicum of products of combustion from a sulfid roasting furnace may be more advantageously used. As stated, the sulfur dioxid in such gases tends to restrain the dissociation of sulfites formed in the oxidation as a 55 preliminary stage to the production of sulfates and it also tends to suppress decomposition of the sulfur trioxid of sulfates into sulfur dioxid and oxygen. Therefore by the use of sulfur dioxid in the draft currents a 60 smooth and perfect conversion of rich galena ores and concentrates into lead sulfate may be effected, enabling, in the case of pure iron-free ores, the production of a cheap white pigment directly from the ore. In this man- 65 ufacture the temperature at no time should

be allowed to rise to the point of fusion or sintering of the ore and the material will remain porous. When ground for paint it will be found to possess great covering power. Sulfate so produced is also well 70 adapted for mixing with a fresh portion of unaltered galena to form lead by the well known reaction.

In forming lead oxid, if it is desired to market it as such, either in the form of litharge or red lead, the oxidation is also preferably so conducted as to avoid fusion or sintering. Red lead may be made in the apparatus shown by finishing the litharge formed in the described way by means of a draft current of hot air. But where the lead oxid is formed as a preliminary to production of lead in the smelter it is desirable to proceed in a slightly different manner. For this purpose while porosity is still desirable, the 80 lumps of ore should nevertheless be sintered more or less to give them some degree of strength and enable them to sustain the weight of the charge in the furnace without breaking down or yielding dust to impede the 85 blast or to be blown out of the furnace. For this purpose the charge of galena should be started to burning in the manner described and oxidation retarded until the reaction has proceeded throughout the mass of the lumps 90 of ore. At this point the dilution of the air draft is discontinued and a sudden evolution of heat permitted throughout the mass, sintering the lumps slightly and giving them 95 mechanical strength. By proper care in the regulation of the draft currents, it is thus possible to produce galena which while sweet roasted, is nevertheless of firm texture. With such proper care it is rarely necessary to use hot air for this finishing but it may be 100 employed if desired.

It is of course, obvious that many other sulfids, such as those of copper, etc., may be roasted in the manner described and I regard my invention as covering the treatment of 105 any sulfid ore or concentrated by this process.

For poor galena where the natural heat of combustion is not great, it is often desirable to work with hot draft currents. It is obvious that my described method gives great latitude to the operator since by changing the degree of the dilution and the temperature of the air, he can either force the heating or slacken it to any desired degree. Perfect 115 control of the operation is given by simple manipulation of valves.

What I regard as novel and desire to claim is:—

1. The process of oxidizing sulfid ores 125 which consists in blowing through an ignited mass of such ore a draft current of diluted air, said air containing controlled proportions of a non-oxidizing diluent.

2. The process of oxidizing sulfid ores 130

which consists in blowing through an ignited mass of such ore a draft current of air diluted with products of complete combustion in controlled proportions.

5 3. The process of oxidizing sulfid ores which consists in blowing through an ignited mass of such ore a draft current of air diluted with carbon dioxid in controlled proportions.

4. The process of oxidizing sulfid ores 10 which consists in blowing through an ignited mass of such ore a draft current of air diluted with controlled proportions of products of complete combustion and a modicum of water vapor.

15 5. The process of oxidizing sulfid ores which consists in blowing through an ignited mass of such ore a draft current of air diluted with controlled proportions of carbon dioxid and with a modicum of water vapor.

20 6. The process of oxidizing galena which consists in blowing through an ignited mass of galena a draft current of diluted air.

7. The process of oxidizing galena which 25 consists in blowing through an ignited mass of galena a draft current of air diluted with products of combustion.

8. The process of oxidizing galena which 30 consists in blowing through an ignited mass of galena a draft current of air diluted with carbon dioxid.

9. The process of oxidizing galena which 35 consists in blowing through an ignited mass of galena a draft current of air diluted with products of combustion and a modicum of water vapor.

10. The process of oxidizing galena which 40 consists in blowing through an ignited mass of galena a draft current of air diluted with carbon dioxid and with a modicum of water vapor.

45 11. The process of oxidizing sulfid ores which consists in igniting a mass of sulfid ore and blowing therethrough a draft current of air diluted to a degree corresponding to the exothermic tendencies to the mass of ore.

12. The process of oxidizing galena which

consists in igniting a mass of galena and blowing therethrough a draft current of air diluted to a degree corresponding to the exothermic tendencies of the mass of ore. 50

13. The process of oxidizing sulfid ores which consists in igniting a mass of such ore, blowing therethrough a current of diluted air until oxidation is nearly complete and then finishing with a draft current of undiluted air to sinter slightly the particles of the roasted mass. 55

14. The process of oxidizing galena which 60 consists in igniting a mass of such ore, blowing therethrough a current of diluted air until oxidation is nearly complete and then finishing with a draft current of undiluted air to sinter slightly the particles of the roasted mass.

15. The process of oxidizing sulfid ores 65 which consists in forcing through an ignited mass of the same a diluted air current of regulated temperature and dilution.

16. The process of oxidizing galena which 70 consists in forcing through an ignited mass of the same a diluted air current of regulated temperature and dilution.

17. The process of oxidizing sulfid ores 75 which consists in forcing through an ignited mass of the same a diluted air current of regulated temperature and dilution and varying said temperature and dilution to agree with the momentary needs of the ore under treatment.

18. The process of oxidizing galena which 80 consists in forcing through an ignited mass of the same a diluted air current of regulated temperature and dilution and varying said temperature and dilution to agree with the momentary needs of the galena under treatments. 85

In testimony whereof I affix my signature, in the presence of two witnesses.

BYRON E. ELDRED.

Witnesses:

HARRY J. TURTON,  
H. M. MARBLE.